

# United States Patent

Metro et al.

[15] 3,671,434

[45] June 20, 1972

[54] **QUINONE PHOSPHATES AS  
LUBRICANT ADDITIVES**

[72] Inventors: **Stephen J. Metro**, Scotch Plains; **Harold  
Shaub**, New Providence, both of N.J.

[73] Assignee: **Esso Research and Engineering Company**

[22] Filed: **Aug. 21, 1970**

[21] Appl. No.: **66,077**

[52] U.S. Cl. .... **252/49.8, 260/964**

[51] Int. Cl. .... **C10m 1/46**

[58] Field of Search..... **252/49.8**

[56]

References Cited

UNITED STATES PATENTS

|           |        |                  |            |
|-----------|--------|------------------|------------|
| 3,558,747 | 1/1971 | Meitsner.....    | 252/49.8 X |
| 2,553,417 | 5/1951 | Ladd et al.....  | 252/49.8 X |
| 2,990,420 | 1/1961 | Gleim et al..... | 252/49.8 X |
| 3,325,567 | 6/1967 | Le Suer.....     | 242/49.8 X |

Primary Examiner—Daniel E. Wyman

Assistant Examiner—W. Cannon

Attorney—Pearlman and Schlager and Carl G. Seutter

[57]

ABSTRACT

Quinone phosphates, including pentoxyphosphoranes, have been found to be effective oxidation and corrosion inhibitors in lubricating oils, especially synthetic ester oils.

11 Claims, No Drawings

## QUINONE PHOSPHATES AS LUBRICANT ADDITIVES

## FIELD OF THE INVENTION

This invention relates to lubricant compositions and more particularly to synthetic oil compositions having improved resistance to deterioration under high performance service conditions. The improved resistance to deterioration may be attributed to the incorporation of quinone phosphate compositions as additives to the lubricant.

## DESCRIPTION OF THE PRIOR ART

The problem of deterioration of lubricating oils and formation of harmful deposits under high performance service conditions has been the cause of much concern in providing satisfactory lubrication of internal combustion engines. This problem is especially acute in lubricating engines of the gas turbine type e.g. turbojet, turboprop and turbofan engines, where lubricants encounter extremely high temperatures. These severe service conditions, which favor oxidation reactions, may break a lubricant down into harmful acidic products which attack the metal parts of the engine or which may act as further oxidation catalysts. The problem is especially serious with regard to magnesium corrosion. Magnesium, which is finding ever-increasing use as a constituent of light-weight metal engines, is especially susceptible to attack by the acidic products of a deteriorated lubricant. In recent years it has been the practice to incorporate into lubricating oils additive compositions to inhibit oxidation and corrosion. Many of these prior art compounds, however, have been found to be unacceptable for use in jet type engines. Investigation has shown that these compounds, at high temperatures, may become extremely corrosive to engine parts.

It is an object of this invention to provide a lubricant additive which is effective as a corrosion and oxidation inhibitor. Other objects will be apparent to those skilled in the art.

## SUMMARY OF THE INVENTION

In accordance with certain of its aspects, this invention is directed to lubricating compositions comprising a major amount of a lubricating oil and a minor corrosion and oxidation inhibiting amount of a quinone phosphate. The quinone phosphates may be characterized by the formula



wherein R and R' may each be a hydrocarbon; Ar is a hydrocarbon radical selected from the group consisting of benzene, naphthalene, pyrene, anthracene, and phenanthrene; and n is an integer 0-4.

## DESCRIPTION OF THE INVENTION

The quinone phosphate compounds which may be used in practice of this invention may be prepared by the reaction of a quinone with a phosphite. The quinone compounds may be:



wherein R' may be a hydrocarbon, Ar' is a quinoid ring derived from a hydrocarbon nucleus selected from the group consisting of benzene, naphthalene, pyrene, anthracene, and phenanthrene nuclei, and n is an integer 0-4.

Preferably Ar' is an anthracene nucleus and the quinone is an anthraquinone:



Typical quinones may include o-quinone, i.e. o-benzoquinone; p-quinone; anthraquinone; alpha or beta naphthaquinone; pyrenediquinone (e.g. 4,5,9,10-pyrenediquinone); 1,4-dihydroxy, anthraquinone (i.e. quinizarin); quinizarin dilaurate; etc., including inertly-substituted quinones, e.g. 2,3-dimethyl-1,4-naphthoquinone; 2-methyl-1,4-naphthoquinone; 2,3-dimethyl-anthraquinone; 2-methoxy-1,4-naphthoquinone; 2-ethyl-1,4-naphthoquinone; 2-propyl-anthraquinone; etc. Inertly-substituted quinones may be employed including those bearing e.g. hydrocarbon, alkoxy, etc. substituents.

These quinones may be reacted with phosphites  $\text{P}(\text{OR})_3$ . In the phosphite  $(\text{RO})_3\text{P}$ , R may be a hydrocarbon moiety, typically alkyl. When R is alkyl, it may be methyl, ethyl, propyl, isopropyl, n-butyl, i-butyl, t-butyl, hexyl, octyl, etc. When R is cycloalkyl, it may be cyclohexyl, etc. The R group may be inertly substituted, i.e. it may bear a substituent which does not react with the other components of the process or interfere with the reaction. Typical inert substituents may include ether, alkyl, etc. Typical inertly-substituted R radicals may include 2-ethyl-hexyl, ethoxyethyl, methylcyclohexyl, etc. All the R groups in a particular compound need not be the same; preferably however, they may be the same. More preferably, R may be alkyl and more preferably, lower alkyl having one to 10 carbon atoms.

Preparation of the additives used in practice of this invention may typically be effected by the reaction of a phosphite (I)  $\text{P}(\text{OR})_3$  with a quinone typically having the following formula:



Reaction may be carried out typically as follows:



or





(I)



(VII)

Preferably reaction may be carried out (q.v., Ramirez et al. 20 *J. Org. Chem.* 33 January 1968, page 20-24) by maintaining the reactants, typically in inert solvent such as benzene, at reflux temperature under nitrogen. After typically 20-24 hours at reflux, the solvent may be evaporated and the typically yellow oil water washed and crystallized. Commonly 25 recrystallization may be effected from a mixture of benzene and hexane.

When  $n$  is other than 0, the quinone compounds may be prepared by the process of U.S. Pat. No. 3,470,099, and the  $OCOR'$  group will preferably be on a ring other than that bearing the quinone structure.

Typical of specific quinone phosphates which may be employed in practice of this invention may be the following:



(VIII)



(IX)



(X)



(XI)



(XII)



(XIII)

35

40

45

50

55

60

65

70

75



(XIV)



(XV)



(XVI)



(XVII)



(XVIII)



(XIX)



(XX)



(XXI)



(XXII)



(XXIII)



(XXIV)



(XXV)



(XXVI)



(XXVII)

4

Although ortho- and para-quinones may be employed, the para-quinones may be preferred. Monoquinones (containing two quinone oxygens) may be preferred, although polyquinones, such as the diquinone 4,5,9,10-pyrenediquinone may be employed.

The orthoquinones, when reacted with the phosphites, may yield phosphorane-ring compounds such as XXVIII - XXXI within the scope of this invention.



The preferred compound may be compound (VIII) 35 prepared by the reaction of anthraquinone and trimethyl phosphate.

A preferred class of quinone phosphates which may be used in practice of this invention may be those prepared from acylated quinones with trialkyl phosphates. Typical of these 40 may be acylated quinizarin:



In these compounds, R' may be selected from the same group as that from which R supra may be selected; but 60 preferably R' may be a long-chain alkyl, preferably containing 8-18 carbon atoms.

These compounds may be prepared by the reaction of a phosphite, such as trimethyl phosphite, with an acylated quinone, such as quinizarin dilaurate. Reaction may be effected by reacting the acylated quinone with an excess of alkyl phosphate at reflux in an inert atmosphere. After reflux for up to 24 hours, the excess phosphite may be stripped off under vacuum; and the residue is dissolved in inert solvent, such as ethyl ether, washed with dilute base, dried, and stripped of solvent.

Although the products appear to be of high purity, based upon elemental and spectroscopic analysis, by-products formed (which need not be removed) may include:



Illustrative compounds in this class may include:

- 15 a. 10-methoxy-9-hydroxyanthracene dimethyl phosphate 1,4-dilaurate;
- b. 10-ethoxy-9-hydroxyanthracene diethyl phosphate 1,4-distearate;
- c. 2-methyl-10-methoxy-9-hydroxyanthracene dimethyl phosphate 1,4-dilaurate;
- d. 4-methoxy-1-hydroxy naphthalene dimethyl phosphate 5,8-dilaurate;
- e. 2-methyl-4-methoxy-1-hydroxy naphthalene dimethyl phosphate 5,8-dilaurate;
- f. 6-methyl-4-methoxy-1-hydroxy naphthalene dimethyl phosphate 5,8-dilaurate;

The preferred compound in this class may be the reaction product of quinizarin dilaurate and trimethyl phosphite:



i.e. 10-methoxy-9-hydroxy anthracene dimethyl phosphate 1,4-dilaurate.

- 45 In practice of the novel process of this invention, the quinone phosphates may be added to the lubricating composition in a minor corrosion and oxidation inhibiting amount. Typically, such an amount may be 0.01 - 5 percent by weight, preferably 0.1-4 weight percent, say 0.1-1 weight percent, 50 typically 0.5 weight percent.

The lubricating oil which may be improved by the technique of this invention may preferably include synthetic ester oils such as high molecular weight, high-boiling liquid aliphatic dicarboxylic acid esters or di- or tri- or tetra-esters of hindered polyols. The viscosity of these oils (when treated in accordance with practice of this invention) may typically be 3.0-8.0 cs at 210° F.

When the base fluid is an ester it may be prepared from various combinations of aliphatic monocarboxylic acids and dicarboxylic acids having from about five to 36 carbon atoms, and monohydric and polyhydric aliphatic alcohols having from about four to about 20 carbon atoms. Specific examples of these esters that may be used are: di-iso-octyl adipate, didecyl azelate, di-isodecyl azelate, di-isodecyl adipate, ditridecyl adipate, di-iso-octyl sebacate, di-isodecyl sebacate, di-2-ethylhexyl sebacate, di-iso-octyl dodecanedioate, di-2-ethylhexyl azelate, and di-2-ethylhexyl adipate. Other esters may also be used as synthetic lubricants that are made from hindered polyols and mono- and polycarboxylic acids of about five to 13 carbon atoms.

The base oil is a hindered polyester having at least two ester linkages per molecule; it therefore includes diesters such as neopentyl glycol dipelargonate and di(2,2,4-trimethylpentyl) sebacate. The term "neutral" is used to mean a fully esterified product.

It is to be understood that in the esterification reaction, there may be used more than one of any of the reactants mentioned e.g. a mixture of monocarboxylic acids, and in any case, the neutral ester product of the esterification reaction will sometimes consist of a mixture of different ester molecules, so the expression "polyester" is to be construed in this light.

Examples of suitable acids and alcohols that may be used in the preparation of the polyester are caprylic acid, capric acid, caproic acid, enanthic acid, pelargonic acid, valeric acid, pivalic acid, propionic acid, butyric acid, 2-ethylhexanoic acid, adipic acid, sebacic acid, azelaic acid, 2,2,4-trimethylpentanol, neopentyl alcohol, neopentyl glycol, trimethylolethane, trimethylolpropane, trimethylolbutane, pentaerythritol and dipentaerythritol.

The most suitable polyesters are the esters of trimethylolpropane, trimethylolbutane, trimethylolethane, pentaerythritol and/or dipentaerythritol with one or more monocarboxylic acids having three to 10 carbon atoms, particularly one or more of those mentioned in the previous paragraph, and more complex esters, for example those prepared from trimethylolpropane, sebacic, adipic, and/or azelaic acid, and one or more monocarboxylic acids having three to 10 carbon atoms, particularly one or more of those mentioned in the previous paragraph.

Illustrative ester-type lubricating oils may include:

TABLE

di-2-ethylhexyl sebacate  
di-2-ethylhexyl azelate  
di-2-ethylhexyl adipate  
di-n-amyl sebacate  
di-2-ethylhexyl-n-dodecyl succinate  
di-2-ethoxyethyl sebacate  
trimethylolpropane tripelargonate  
trimethylolpropane tricaproate  
trimethylolpropane tricaprylate  
trimethylolpropane tri-neoheptanoate  
trimethylolpropane tri-neodecanoate  
trimethylolpropane mono-neoheptanoate dipelargonate  
di(C<sub>n</sub>-C<sub>10</sub>-oxoalcohol) adipate  
tetra (C<sub>5-10</sub> monocarboxylic acid) esters of pentaerythritol

These oils may be blended with other oils, such as castor oil; lard oil; polymerized olefins; copolymers of alkyleneglycols or aliphatic alcohols with organic acids, etc.

The additives of the present invention may be used alone or preferably in combination with other additives in a lubricating composition. These other additives, typically present in amount of 0.001 - 10 weight percent each may include:

- oxidation inhibitors such as aromatic amines e.g. phenothiazine;
- metal corrosion inhibitors such as benzotriazole;
- load-carrying agents, such as tricresyl phosphate;
- anti-foamants such as a silicone;
- dispersants such as the polymethacrylates.

The novel compositions of this invention may include concentrates of quinone phosphates (which may be added to lubricating compositions) in inert diluents including lubricating compositions, solvents, e.g. esters, in amount of 10 - 90 percent; and these concentrates may include other additives.

Addition of quinone phosphate to lubricating oils in accordance with the technique of this invention permits attainment of outstanding results when the composition is subjected to The Oxidation Corrosion Stability Test which is carried out by suspending metal pieces in oil. Dry air is bubbled at 5 liters per hr. through 100 g. of oil at 425° F. for 72 hours. These tests simulate to a degree the operating conditions of jet engines. At the end of the test, the following may be determined:

- the corrosion of each metal tested in mg/cm<sup>2</sup>;
- the percent increase in centistoke viscosity; and
- the increase in total acid number (TAN).

This OCS Test is similar to Military Specification MIL-L-7808-G except that the OCS test is run at 425° F. instead of 347° F.

In typical Oxidation Corrosion Stability Tests it may be found that use of the novel systems of this invention permits attainment of substantially decreased weight loss for magnesium under severe oxidative conditions.

It may also be found that the increase in total acid number (TAN) is substantially smaller than that attained without use of the additives of this invention. Commonly it is found that the % Δ kinematic viscosity is significantly reduced by the use of the instant invention.

#### DESCRIPTION OF PREFERRED EMBODIMENTS

##### Examples I-IV

- In these examples, which represent a preferred embodiment of the invention, the quinone phosphate (Compound A) was prepared from a commercially-available hydrocarbon mixture, having an average molecular weight of about 300, and containing substantial proportions of alkylated aromatics. This composition may be oxidized to form the corresponding quinone by the method of U.S. Pat. No. 2,373,003 to Arnold.
- In this oxidation, 100 g. of alkylated aromatic may be mixed with 1,000 ml. of glacial acetic acid, 500 ml. of 30 percent hydrogen peroxide added dropwise over a 30-minute period, and the reaction mixture refluxed for 22 hours. The acetic acid and water was then stripped under vacuum.
- The crude reaction product was dissolved in 1000 ml. of ethyl ether, the mixture filtered and washed with 3 × 250 ml. of 5 percent sodium bicarbonate solution, followed by 2 × 250 ml. water.
- The resulting ether solution was dried and the ether stripped. 70.3 g. of product was obtained. The lower phase of the product mixture, 48.8 g. was separated. Infrared analysis showed presence of quinone structure.
- 48.8 g. of this product was mixed with 125 g. (1 mole) of trimethyl phosphite; and the mixture was refluxed for 24 hours under a blanket of nitrogen. The excess of trimethyl phosphite was stripped off under vacuum. The crude reaction product was dissolved in 1,000 ml. anhydrous ethyl ether. The ether solution was twice washed each time with 250 ml. of aqueous sodium bicarbonate and then twice with 250 ml. water. The ether solution was then dried, and the ether removed by evaporation under nitrogen. The product was then vacuum desiccated for 12 hours to remove remaining traces of water and ether. The product, Compound A, was obtained in yield of 40 grams.

The Base Lubricating Oil which was employed contained the following:

| Parts | Component                                                                    |
|-------|------------------------------------------------------------------------------|
| 70    | Trimethylol propane ester of C <sub>n</sub><br>average monocarboxylic acids. |
| 30    | Dipentaerythritol ester of C <sub>n</sub><br>average monocarboxylic acids.   |
| 1.3   | p,p'-Diictio diphenyl amine.                                                 |
| 1.1   | Phenyl α-naphthylamine.                                                      |
| 0.1   | Benzotriazole.                                                               |
| 0.02  | Sebacic acid.                                                                |
| 0.001 | Silicone.                                                                    |

With the base oil, the following compositions were formulated:

- Base oil alone;
  - Base oil, 100 parts, plus 3 parts tricresyl phosphate a commercial additive;
  - Base oil, 100 parts, plus 0.05 parts of Compound A;
  - Base oil, 100 parts, plus 0.1 parts of Compound A.
- The OCS test was carried out and the weight loss of magnesium, the change in viscosity, and the TAN determined.

TABLE

| Oil | Metal weight loss, mg./cm. <sup>2</sup> |        |       |       |       |       |
|-----|-----------------------------------------|--------|-------|-------|-------|-------|
|     | Cu                                      | Mg     | Fe    | Al    | Ag    | Ti    |
| I   | -1.80                                   | -11.74 | +0.01 | +0.01 | -0.01 | +0.01 |
| II  | -0.11                                   | -10.23 | +0.03 | +0.03 | 0.00  | +0.03 |
| III | -0.04                                   | -1.50  | +0.04 | +0.01 | -0.01 | +0.02 |
| IV  | -0.14                                   | -1.87  | +0.06 | +0.01 | 0.00  | +0.01 |

NOTE.—425° F. 72 hour OCS test.

From this table, it will be apparent that the weight loss of magnesium is desirably decreased. Although the base oil alone permitted a loss of 11.74 mg/cm<sup>2</sup>, use of the technique of this invention in Example III permitted a loss of only 1.50 mg/cm<sup>2</sup>, i.e. a drop to only 12.7 percent (a tenfold reduction) of that recorded with the base oil alone. Simultaneously the weight losses with copper, iron, aluminum, silver, and titanium all were either bettered (i.e. decreased) or desirably showed little or no change.

#### Examples V-XII

In Examples V and VI, which represent a more preferred embodiment of the invention, the quinone phosphate (Compound B) was quinizarin dilaurate phosphate product prepared by the reaction of (a) one mole of quinizarin dilaurate (i.e. 1,4-dilauroyl-9,10-anthraquinone) and (b) one mole of trimethyl phosphite.

Specifically 63.4 g. (0.1 mole) of quinizarin dilaurate was dissolved in 125 g. (1 mole) of trimethyl phosphite in a reaction vessel. The mixture was refluxed for 24 hours under a blanket of nitrogen. The excess of trimethyl phosphite was then stripped off under vacuum. The crude reaction product was dissolved in 1,000 ml. anhydrous ethyl ether. The ether solution was twice washed, each time with 250 ml. of aqueous sodium bicarbonate and then twice with 250 ml. of water. The ether solution was then dried, and the ether removed by evaporation under nitrogen. The product was then vacuum dessicated for 12 hours to remove remaining traces of water and ether.

In Examples VII and VIII, the quinone phosphate (Compound C) was the quinizarin dioctanoate phosphate product prepared by the reaction of (a) one mole of quinizarin dioctanoate and (b) one mole of trimethyl phosphite. This product was prepared by the same process as that of Examples V and VI except that the charge material was quinizarin dioctanoate.

The following compositions were formulated:

- V. Base oil, 100 parts, plus 0.1 parts of Compound B.
- VI. Base oil, 100 parts, plus 0.05 parts of Compound B.
- VII. Base oil, 100 parts, plus 0.1 parts of Compound C.
- VIII. Base oil, 100 parts, plus 0.5 parts of Compound C.
- IX. Base oil, 100 parts, plus 0.05 parts quinizarin dilaurate.
- X. Base oil, 100 parts, plus 0.1 parts quinizarin dilaurate.
- XI. Base oil, 100 parts, plus 0.1 parts quinizarin dioctanoate.
- XII. Base oil, 100 parts, plus 0.5 parts quinizarin dioctanoate.

When these compositions were subjected to the OCS test, supra, the following were noted. Examples I and II are repeated for convenience. It will be noted that Example II is reported in quadruplicate, and Examples V and VI in duplicate.

#### 425° F. OXIDATION-CORROSION STABILITY TEST (OCS) 72 HOURS

| Oil  | New oil |      | Metal weight loss, mg./cm. <sup>2</sup> |        |       |       |       | Used oil |        | Percent<br>ΔKV/100 | Δtan   |      |
|------|---------|------|-----------------------------------------|--------|-------|-------|-------|----------|--------|--------------------|--------|------|
|      | KV/100  | Tan  | Cu                                      | Mg     | Fe    | Al    | Ag    | Ti       | KV/100 | Tan                |        |      |
| I.   | 26.34   | 0.30 | -1.80                                   | -11.74 | +0.01 | +0.01 | -0.01 | +0.01    | 279.2  | 4.33               | 959.98 | 4.03 |
|      | 25.75   | 0.39 | -0.09                                   | -9.78  | +0.01 | +0.02 | -0.01 | +0.02    | 39.72  | 4.47               | 54.25  | 4.08 |
| II.  | 25.86   | 0.39 | -0.18                                   | -7.92  | +0.03 | 0.00  | -0.01 | +0.01    | 39.63  | 6.09               | 53.25  | 5.70 |
|      |         |      | -0.11                                   | -12.20 | +0.03 | 0.00  | +0.01 | +0.01    | 40.44  | 4.75               |        |      |
| V.   | 26.44   | 0.39 | -0.11                                   | -10.23 | +0.03 | +0.03 | 0.00  | +0.03    | 40.17  | 4.33               |        |      |
|      | 26.50   | 0.39 | -0.15                                   | -5.05  | +0.02 | 0.00  | -0.01 | +0.01    | 37.68  | 4.26               | 42.51  | 3.87 |
| VI.  |         |      | -0.12                                   | -8.7   | +0.02 | +0.01 | -0.03 | 0.00     | 38.85  | 5.43               | 46.60  | 4.76 |
|      |         |      | -0.13                                   | -0.40  | +0.02 | +0.01 | -0.04 | 0.00     | 38.40  | 7.18               |        |      |
| VII. | 26.55   | 0.34 | -0.17                                   | -1.47  | +0.03 | 0.00  | -0.09 | 0.00     | 37.23  | 6.25               | 40.23  | 5.91 |
|      | 26.92   | 0.49 | -0.15                                   | -0.09  | +0.03 | +0.01 | -0.01 | 0.00     | 36.66  | 6.04               | 36.18  | 5.55 |
| IX.  | 26.33   | 0.36 | -1.15                                   | -11.06 | -0.01 | +0.01 | -0.01 | -0.01    | 123.4  | 5.32               | 368.67 | 4.96 |
|      | 26.27   | 0.37 | -0.96                                   | -8.01  | -0.01 | +0.01 | -0.01 | -0.01    | 116.2  | 4.76               | 342.33 | 4.39 |
| X.   | 26.37   | 0.31 | -0.74                                   | -10.02 | +0.01 | +0.01 | -0.01 | -0.01    | 123.3  | 5.12               | 367.58 | 4.81 |
|      | 26.55   | 0.38 | -0.26                                   | -12.53 | -0.01 | +0.01 | -0.01 | -0.01    | 113.3  | 6.21               | 326.74 | 5.83 |

From the above table, it will be noted that the weight loss for magnesium in Example V is about half that of control Examples I-II. More unexpectedly, the weight loss for magnesium in Examples VI-VIII is substantially lower; and the loss in Example VIII is outstandingly low.

The weight loss for other metals in Examples V-VII is also characterized as low and well within the specified limits.

Unexpectedly it is noted that the change in kinematic

viscosity is very low: 36.18 to 46.60 percent in contrast to 959.98 percent for Example I and 53-54 percent for Example II.

The change in Total Acid Numbers is well within the desired limits (below 6).

It will be apparent that Examples IX-XII, using quinizarin dilaurate and quinizarin dioctanoate, not within the scope of this invention, yielded results which were unsatisfactory — particularly with respect to:

- 10 a. copper and magnesium corrosion; and
- b. viscosity increase.
- 15 a. satisfactory initial and final viscosity;
- b. satisfactory initial and final acid number;
- c. satisfactory oxidation-corrosion properties with respect to copper, iron, aluminum, silver, and titanium; and
- d. outstanding reduction (almost elimination) of oxidation-corrosion of magnesium.

20 In other comparative OCS tests (under standard specification MIL-L-23699) carried out at 400° F., it was observed that the loss of copper from a copper coupon averaged 2.49 mg/cm<sup>2</sup> in the presence of base oil alone, 0.035 mg/cm<sup>2</sup> in the presence of base oil containing quinizarin dilaurate-methyl phosphate, and 0.36 mg/cm<sup>2</sup> in the presence of base oil containing the same amount of quinizarin dilaurate.

25 In the case of a magnesium coupon, the corresponding numbers were 0.19, 0.015, and 0.17.

30 The percent change in viscosity was found similarly to be 36.1, 19.7, and 26.2.

35 From these data, it may be concluded that the base oil containing quinizarin dilaurate-methyl phosphate of this invention reduces copper corrosion by a factor of 10 (as compared to quinizarin dilaurate alone) and by a factor of about 70 (as compared to the base oil alone).

40 Similarly the base oil containing quinizarin dilaurate-methyl phosphate of this invention reduces magnesium corrosion by a factor of 10 (as compared to quinizarin dilaurate alone) and by a factor of 10 (as compared to the base oil alone).

45 In the case of viscosity, it was noted that the Base Oil and the Base Oil containing quinizarin dilaurate were above the set specification of 25 (%Δ viscosity at 100° F. measured after the 400° F. test) of MIL-L-23699. The percent viscosity change of the Base Oil containing quinizarin dilaurate-methyl phosphate was 19.7 percent — which is well below the maximum specification of 25 percent set by specification MIL-L-23699.

50 Thus, it will be noted that practice of this invention yields a product which is eminently satisfactory in the respect to the

parameters of the 400° F. oxidation test — while the Base oil alone or containing e.g. quinizarin dilaurate fails on these counts.

70 The lubricating oils which may be improved by the technique of this invention may be synthetic ester oils, preferably high molecular weight, high-boiling ester oils formed typically from an aliphatic, carboxylic acid and preferably a hindered polyol. Such oils may commonly have a

viscosity (when treated by the process of this invention) of 3.0 - 8.0 cs at 210° F.

The lubricating oil may be a synthetic ester oil formed by the reaction of a C<sub>5</sub>-C<sub>36</sub> acid and a C<sub>4</sub>-C<sub>20</sub> alcohol. According to one aspect of this invention, the oil may preferably be formed from (a) a C<sub>3</sub>-C<sub>36</sub> aliphatic acid R(COOH)<sub>n</sub> wherein R is an aliphatic hydrocarbon (including inertly-substituted hydrocarbon) residue and n is typically 1-3 and (b) a C<sub>4</sub>-C<sub>20</sub> aliphatic alcohol R'(OH)<sub>m</sub> wherein R' is an aliphatic hydrocarbon (including inertly-substituted hydrocarbon) residue and m is an integer preferably 1-6, most preferably 1-3.

The base oil may, in one embodiment, be a liquid ester product of an aliphatic monocarboxylic acid and a polyol. Preferably the aliphatic monocarboxylic acid may have the formula R(COOH) wherein R is an aliphatic hydrocarbon moiety.

The preferred of these acids may be C<sub>3</sub>-C<sub>36</sub>, preferably C<sub>5</sub>-C<sub>10</sub> acids. Typical of such acids may be:

|                      |                 |
|----------------------|-----------------|
| caproic acid         | C <sub>6</sub>  |
| caprylic acid        | C <sub>8</sub>  |
| capric acid          | C <sub>10</sub> |
| enanthic acid        | C <sub>11</sub> |
| pelargonic acid      | C <sub>9</sub>  |
| valeric acid         | C <sub>5</sub>  |
| pivalic acid         | C <sub>5</sub>  |
| propionic acid       | C <sub>3</sub>  |
| butyric acid         | C <sub>4</sub>  |
| 2-ethylhexanoic acid | C <sub>8</sub>  |

The polyols which may be reacted with the noted aliphatic monocarboxylic acids, to form esters, may include R'(OH)<sub>m</sub> wherein R' is an aliphatic moiety and m is an integer preferably 2-6, more preferably 2-4. The preferred polyols may be the C<sub>2</sub>-C<sub>6</sub>, say C<sub>2</sub>-C<sub>4</sub> polyols. Typical of such polyols may be:

|                     |
|---------------------|
| neopentyl glycol    |
| trimethylol ethane  |
| trimethylol propane |
| trimethylol butane  |
| pentaerythritol     |
| dipentaerythritol   |

Typical esters of aliphatic monocarboxylic acids and polyols may be



including the following illustrative examples:

TABLE

|                                        |  |
|----------------------------------------|--|
| pentaerythritol tetra-valerate         |  |
| pentaerythritol tetra-caproate         |  |
| pentaerythritol tetra-2-ethylhexanoate |  |
| pentaerythritol tetra-pelargonate      |  |
| pentaerythritol tetra-butyrate         |  |
| dipentaerythritol hexa-valerate        |  |
| dipentaerythritol hexa-pelargonate     |  |
| dipentaerythritol hexa-caprate         |  |
| trimethylol propane tri-caproate       |  |
| trimethylol propane tri-butyrate       |  |
| trimethylol propene tri-valerate       |  |
| trimethylol propane tri-pelargonate    |  |

In another embodiment, the base oil may be a liquid synthetic ester product of an aliphatic polycarboxylic acid and an aliphatic monohydroxy alcohol.

Preferably the aliphatic polycarboxylic acid may have the formula R(COOH)<sub>n</sub> wherein n is greater than 1 and preferably 2-3. Typical polycarboxylic acids may include:

|                 |
|-----------------|
| adipic acid     |
| azelaic acid    |
| sebacic acid    |
| dodecanoic acid |

Illustrative of the esters so formed may be: di-2-ethylhexyl sebacate; di-2-ethylhexyl adipate; di-2-ethylhexyl azelate; di-C<sub>n</sub>-oxo alcohol sebacate; di-2-ethylbutyl pivalate; and di-3,5-trimethyl adipate.

Although this invention has been illustrated by reference to

75

specific embodiments, it will be apparent to those skilled in the art that various changes and modifications may be made which clearly fall within the scope of this invention.

What is claimed is:

1. A lubricating composition comprising:
- a. a major amount of lubricating oil; and
- b. a minor corrosion and oxidation inhibiting amount of a phosphate of a hydroquinone having the formula:



wherein R and R' are each a hydrocarbon; Ar is selected from the group consisting of benzene, naphthalene, pyrene, anthracene, and phenanthrene, and n is an integer 0-4.

2. A lubricating oil composition as claimed in claim 1 wherein the lubricating oil is a synthetic ester lubricating oil.

3. A lubricating composition as claimed in claim 1 wherein n is 0.

4. A lubricating composition as claimed in claim 1 wherein n is 2.

5. A lubricating composition as claimed in claim 1 wherein R is a C<sub>1</sub> to C<sub>10</sub> alkyl group and R' is a C<sub>8</sub> to C<sub>18</sub> long-chain alkyl group.

6. A lubricating composition as claimed in claim 1 wherein said compound is



wherein R and R' are each a hydrocarbon; and n is an integer 0-4.

7. A lubricating composition as claimed in claim 1 wherein said compound is:



8. A lubricating composition as claimed in claim 1 wherein said compound is:



wherein R and R' are each a hydrocarbon.

9. A lubricating composition as claimed in claim 1 wherein said compound is:

**13****14**

11. A lubricating composition as claimed in claim 1 wherein said compound is



10. A lubricating composition as claimed in claim 1 wherein  $n$  is 2 and  $R'$  is  $C_8$  to  $C_{18}$ .

5

10

15

\* \* \* \* \*

20

25

30

35

40

45

50

55

60

65

70

75